

[54] PROCESS FOR THE REMOVAL OF THIOLS  
FROM HYDROCARBON OILS

[75] Inventors: Robert L. Jacobson, Hercules; Kirk  
R. Gibson, El Cerrito, both of Calif.

[73] Assignee: Chevron Research Company, San  
Francisco, Calif.

[\*] Notice: The portion of the term of this patent  
subsequent to Jul. 24, 1996, has been  
disclaimed.

[21] Appl. No.: 915,022

[22] Filed: Jun. 12, 1978

Related U.S. Application Data

[63] Continuation-in-part of Ser. No. 892,544, Apr. 3, 1978,  
Pat. No. 4,163,708.

[51] Int. Cl.<sup>2</sup> ..... C10G 29/16; C10G 29/06;  
C10G 29/04

[52] U.S. Cl. ..... 208/243; 208/89;  
208/246; 252/419

[58] Field of Search ..... 208/243, 246, 89, 245

[56]

References Cited

U.S. PATENT DOCUMENTS

2,755,227 7/1956 Lucas ..... 208/89  
4,113,606 9/1978 Mulaskey ..... 208/246

FOREIGN PATENT DOCUMENTS

2119803 8/1972 France ..... 208/246

Primary Examiner—George Crasanakis  
Attorney, Agent, or Firm—D. A. Newell; R. H. Davies;  
R. H. Evans

[57]

ABSTRACT

Thiol impurities are absorbed and removed from hydrocarbon oils by contacting the oil in the absence of molecular oxygen with a scavenger at a temperature in the range of about 120° to 400° C. The scavenger is a composite having a copper component and an inorganic porous carrier component and having a surface area in the range 20 to 1000 square meters per gram. The contacting must be discontinued when the thiol impurity content of the effluent product exceeds about 0.3 ppm.

13 Claims, No Drawings

PROCESS FOR THE REMOVAL OF THIOLS  
FROM HYDROCARBON OILS

CROSS REFERENCE TO RELATED  
APPLICATION

This application is a continuation-in-part of U.S. Ser. No. 892,544, filed Apr. 3, 1978, which issued as U.S. Pat. No. 4,163,708.

BACKGROUND OF THE INVENTION

This invention relates to a process for improving a hydrocarbon oil by removing thiol sulfur from the oil. More particularly, it relates to the removal of such sulfur by contacting the oil with a copper-containing scavenger under suitable conditions.

PRIOR ART

It is known in the art to improve a thiol-containing hydrocarbon stream by converting the thiol impurity to a relatively "sweet" organic disulfide (see for example U.S. Pat. Nos. 2,755,226 and 2,769,764). It is also known to improve a thiol-containing hydrocarbon stream by oxidizing the thiol components of the stream using molecular oxygen and a copper-containing oxidation catalyst (see for example U.S. Pat. Nos. 2,338,371, 2,653,125 and 3,192,152). In these processes, the thiol is converted to the disulfide which is included in the product obtained from the process. Thus in both of the foregoing processes, only the form of the sulfur is changed and relative to sulfur impurity content, the resulting product remains objectionable on the basis of its sulfur content. Under contemporary environmental standards, the presence of sulfur in a hydrocarbon, particularly where it is to be used as a fuel, is undesirable because of the sulfur content of the exhaust from combustion of the fuel.

In a yet further process for the improvement of hydrocarbon oils by sweetening, it is known to convert thiol impurities to oil-soluble copper mercaptides under ambient or moderate temperature condition and to remove these mercaptides from the hydrocarbon oil by contact with a suitable absorbent, for example, a heavy metal sulfosilicate, pumice, clay, silica gel, keiselguhr, Fuller's earth, boria, and the like. The presence of oil-soluble copper compounds in a hydrocarbon oil is undesirable for a variety of reasons, including: (1) a destabilizing effect which copper compounds have upon hydrocarbon oils on standing; and (2) where the oil is to be subjected to downstream processing using a catalyst, copper impurities often exert deleterious effects upon the catalyst, for example, the activity of a platinum reforming catalyst is seriously reduced by copper contamination.

SUMMARY OF THE INVENTION

The present invention is a process for absorbing thiol impurity from a hydrocarbon oil boiling below about 300° C., preferably in the range from about 10° C. to about 300° C., having a total sulfur-containing-impurity content, calculated as elemental sulfur, in the range below about 1000 ppm, including at least 0.4 ppm (calculated as sulfur) of thiol impurity, which comprises contacting the oil in the substantial absence of molecular oxygen with a scavenger at a temperature in the range from about 120° to 400° C. The scavenger comprises an essentially oil-insoluble solid composite having a copper component and an inorganic porous carrier

component and having a surface area in the range from about 20 to 1000 square meters per gram. The copper component is selected from the group consisting of copper metal and copper compounds. The carrier component is selected from the group consisting of refractory metal oxides or mixtures thereof or carbon. The contacting is continued so long as the resulting effluent oil has a thiol content below about 0.3, preferably 0.2 ppm. Thus for practical purposes, the resulting product is virtually free of thiol impurity.

Such a product is especially desirable for use as feed to hydrocarbon reforming process (see, for example, U.S. Pat. No. 3,415,737—H. E. Kluksdahl) using a platinum-rhenium-alumina catalyst or to a hydrogen gas producing process using nickel oxide catalyst, especially where the sulfur-containing impurity prior to the contacting consists essentially of thiol. Even a reduction in thiol sulfur content from 1 ppm to 0.1 ppm results in remarkable catalyst life improvements. In reforming, surprisingly, this improvement is usually in the 25-50 percent range, and may even be as high as 200 percent depending upon the severity of the reforming conditions.

By the term "thiol sulfur" as used herein is meant combined sulfur contained in thiol molecules, RSH, where R is a hydrocarbon radical.

EMBODIMENT

In a preferred embodiment, a medium-boiling-range gasoline naphtha containing, as substantially its sole sulfur-containing impurity, about 1 ppm of thiol impurity is treated for use as feed to a reformer. Virtually all (that is, within the limits of experimental accuracy, a residual thiol content of about 0.1 ppm) of this impurity is removed (absorbed) from the naphtha. The removal is accomplished by contacting the naphtha with a suitable scavenger in a contacting zone under conditions including, as follows:

|                              |     |
|------------------------------|-----|
| Temperature, °C.             | 165 |
| Pressure, Atm. Abs.          | 11  |
| Liquid Hourly Space Velocity | 10  |

The scavenger is a composite of copper chromite disposed upon porous alumina having a surface area of about 200 square meters per gram and a copper chromite content, calculated as copper metal, of about 14 weight percent. The contacting is continued so long as the resulting product stream has a sulfur content below a predetermined value, for example, 0.3 ppm, preferably 0.1 ppm. In addition to the thiol impurity, any traces of hydrogen sulfide which may be present in the naphtha, for example, because of incomplete removal in a previous gas stripping or distillation step, is also virtually all removed. Under comparable reforming conditions and using a comparable platinum-rhenium-alumina reforming catalyst, the catalyst life using the above-treated feed exhibits an end-of-run life which is greater than that using the untreated feed by at least about fifty percent, and usually in the 50-150 percent range. The economical value of the treatment is large. The scavenging is desirably controlled by monitoring the sulfur content of the effluent product stream and discontinuing the contacting when the thiol-sulfur content, calculated as elemental sulfur exceeds the predetermined value.

The above scavenging of the thiol impurity has a number of advantages: (1) it effectively reduces thiol

impurity content of a reformable naphtha feed; and (2) it accomplishes this desirable result without having to subject the feed to additional expensive hydrogenating stages under conditions of diminishing returns (un-avoidable recombination of olefin-H<sub>2</sub>S products to thiol).

#### Thiol-Sulfur End Point

The scavengers of the present invention have been found to effectively absorb thiols, particularly higher-molecular-weight thiols, e.g., C<sub>5</sub>+ thiols, from relatively dilute thiol-containing hydrocarbon streams. And the absorption remains effective, that is an effluent stream is produced which usually contains less than about 0.1 ppm of thiol sulfur, until 80-99% of the thiol-sulfur capacity of the scavenger has been satisfied. Thereafter the thiol content of the effluent stream rises rapidly and approximates the corresponding value for the feed stream. In effect the scavenger is titrated with the thiols of the feed, and the end point is the appearance of an increasingly appreciable amount of thiol sulfur in the effluent stream. Control of the process is conveniently carried out by monitoring the sulfur content of the effluent product stream using ordinary analytical methods for the determination. Where the feed stream contains an appreciable amount of a sulfur-containing impurity whose source is other than thiol, for example thiophenes, organic sulfides (RSR) or the like, the effluent product stream has a sulfur content which substantially corresponds to the amount of this non-absorbable material present in the feed. The end point for thiol absorption for such a feed will be an increase in the sulfur content of the effluent stream of about 0.3 ppm.

#### The Scavenger

A satisfactory scavenger for the present process should be essentially insoluble in hydrocarbon oils at the contact temperature employed. Otherwise a tradeoff of one impurity for another is made. Therefore the components of the scavenger, for example, the copper and carrier components, should be essentially insoluble (i.e., for practical purposes no appreciable solubility) in hydrocarbon oils in general, and in particular in the process feeds contemplated herein. Scavengers, in general, which satisfy these requirements are contemplated for use in the present process.

A satisfactory scavenger must also have a substantial surface area. Otherwise the number of available thiol absorption sites is too small. Usually when the carrier component or the scavenger per se has a surface area (B.E.T. method) of at least about 20 square meters per gram, sufficient sites will be available for efficient removal of thiol from the process feed. In general, a satisfactory surface area is in the range 20-1000 square meters per gram; preferably it is above about 200 square meters per gram.

#### The Copper Component

A wide variety of copper components are satisfactory for use in the present process. In general, copper metal and copper compounds essentially insoluble in hydrocarbon oils are satisfactory for use herein and are contemplated for such use. The choice of component, in general, will depend upon matters of convenience, for example, relative ease of the incorporating of the component into or onto the surface of the composite which is the scavenger, for example by impregnation, copre-

cipitation and the like ordinary means, and, of course, cost factors. Preferably the copper component is at least one of the group consisting of copper metal, copper oxides and copper compounds convertible to copper oxides by ordinary calcination and/or oxidation methods.

Representative copper components suitable for use herein include copper metal, copper compounds such as oxides, phosphate, chromite, chloride, bromide, fluoride, carbonate, molybdate, hydroxide, complex ammonia-containing compounds and the like copper compounds. The relative amounts of the copper and carrier components satisfactory for use herein varies depending upon the particular combination of carrier and copper component employed. In general, the scavenger will contain a major amount of the carrier and a minor amount of the copper component. Usually an effective amount of the copper component, based upon the total weight of the scavenger, is in the range from about 1 to 20 weight percent, calculated as elemental copper, with the balance of the scavenger comprising the carrier component.

#### The Carrier Component

In general, inorganic materials which are solids at the contact temperature of the present process, which are substantially insoluble in hydrocarbon oils and which have a surface area of at least about 20 square meters per gram are satisfactory for use herein and are contemplated for such use. Preferably the carrier component is selected from the group consisting of carbon, the synthetic and natural refractory oxides of metals of Groups II, III and IV of the Periodic Chart of the Atoms (the Welch Scientific Company) and mixtures thereof. More preferably the carrier component consists essentially of alumina or carbon.

Representative carrier components include alumina, silica, carbon, silica-alumina, boria, kieselguhr, processed diatomaceous earths of commerce, pumice, silicates, and the like having an adequate surface area.

#### The Feed

Petroleum refinery hydrocarbon streams and hydrocarbon oils, in general having a total sulfur-impurity content, calculated as elemental sulfur, in the range below 1000 ppm, including an appreciable (i.e., about 0.4 ppm) thiol-sulfur content and boiling in the range from about 10° C. to about 300° C., are satisfactory as feeds for the present process and are contemplated for use herein. Preferably the stream is one having a sulfur-impurity content below 100 ppm in which the impurity consists essentially of thiol having a carbon atom content in about the C<sub>5</sub>+ range. In the latter case the present process, in general, results in an effluent product stream having little (i.e., below about 0.1 ppm) or no sulfur content.

The presence of dissolved oxygen in the hydrocarbon oil is undesirable because roughly to the extent such oxygen is present at the contacting of the feed with the scavenger, organic disulfide is formed from the thiols present in the feed. Disulfide may be carried along in the resulting effluent product stream. In this case the scavenger is acting as a catalyst to promote oxidation of the thiol rather than as an absorbent. Similarly, there should be little or no molecular oxygen present from any other possible source at the contacting of the feed with the scavenger and for the same reasons.

Representative hydrocarbon feeds satisfactory for use in the present process include straight run and refined petroleum naphthas, hydrocrackate product streams and fractions thereof, diesel oil, jet fuel oil, kerosene and the like hydrocarbon streams having the sulfur impurity and boiling point characteristics as discussed above. In a most preferred aspect of the present invention, the feed to the present process is one which after being subjected to the present treatment is to be subjected to catalytic reforming over a platinum-containing or a bimetallic reforming catalyst.

#### Process Conditions

The contacting of the hydrocarbon feed stream may be carried out in any suitable manner with the hydrocarbon in the liquid or gaseous state or in mixtures thereof and with the scavenger in the fixed-bed or fluid-bed aspect and under ordinary fixed-bed or fluid-bed contacting conditions. Preferably the feed is in the liquid phase, under which condition the higher-molecular-weight thiols are very effectively removed.

##### A. Temperature

Temperatures satisfactory for use in the present process vary over a considerable range. In general a temperature in the range 120° to 400° C. will be satisfactory. Preferably the temperature is in the range 130°-200° C. and more preferably is about 165° C.

##### B. Pressure

In general a suitable pressure will depend upon whether or not the hydrocarbon feed at the contacting is in the liquid or gaseous phase. In the former case, the pressure necessarily must be at least sufficient to maintain the desired liquid phase. Preferably, the contacting is effected at a pressure sufficient to maintain at least the major portion of the feed in the liquid phase.

##### C. Contact Time

The contact time desirably used in the present process varies depending upon a number of factors, including the particle size, the surface area and pore size of the porous carrier used in the preparation of the scavenger, the relative amount of thiol sulfur present in the hydrocarbon feed and the like. In general, a satisfactory contact time will result when the liquid hourly space velocity (LHSV) is in a range from about 0.1-50, preferably 1-40, and the average particle diameter of the carrier is in the range from about 0.004 to 7 mm, preferably 0.7 to 6 mm.

#### Scavenger Regeneration

The scavengers of the present invention, after becoming spent in service by reaching the thiol end point, may be regenerated in any suitable manner. Whether or not it is desirable to regenerate the scavenger is a matter of economics and of the availability of materials required to manufacture a replacement scavenger. Where the scavenger is to be regenerated, it is especially desirable that it contain a catalytic oxidizing component, for example, chromium in the chromite or oxide form, a molybdenum oxide, or the like. Such a component appears to facilitate oxidation of the sulfur impurity. The regeneration is desirably carried out in the following stages:

1. Stripping adhering hydrocarbon from the scavenger;

2. Subjecting the spent scavenger to oxidizing conditions in the presence of molecular oxygen; and

3. Subjecting the oxidized scavenger to reducing conditions in the presence of molecular hydrogen gas.

5 In stripping the adhering hydrocarbon from the spent scavenger, a suitable agent is a gas such as nitrogen, hydrogen, steam or carbon dioxide. The stripping is conveniently carried out at a temperature reasonably approximate to the temperature employed for the thiol absorption stage, for example as in the embodiment described above at about 165° C. To facilitate prompt evaporation of the adhering hydrocarbon, the system pressure is desirably reduced. When the effluent gas stream from the stripping is more or less free of hydrocarbons, the spent scavenger is ready for the next stage of the regeneration.

10 The purpose of the oxidizing stage in the regeneration of the spent scavenger is twofold: (i) to oxidize residual carbon and hydrocarbon containing materials adhering

20 to the scavenger; and (ii) to oxidize the residual sulfur in whatever form present. For this purpose a dilute molecular oxygen-containing gas stream is employed, for example one which contains from 1 to 2 volume percent of molecular oxygen. The reason that a dilute molecular

25 oxygen gas stream is employed is to avoid and to control the exothermic heat of reaction which accompanies the desired oxidations. In this way a "slow burn" is obtained and the temperature of the spent scavenger is maintained at a reasonable level, for example in the range from about 190° to 260° C. The oxidation is complete when the effluent gas stream has substantially the same composition as the feed stream employed for the oxidation stage.

30 For the final stage of the regeneration, the oxidized spent scavenger is desirably purged using a stream of nitrogen gas in order to remove most if not all of the molecular oxygen gas remaining in the scavenger. The purpose of the reducing stage is to convert the metal sulfur oxide moiety present in and/or on the scavenger

35 to sulfur dioxide, which is carried away in the effluent gas stream leaving the copper component of the scavenger in the form of copper oxide and/or copper metal. The reducing stage of the regeneration is complete when for practical purposes the effluent gas stream

40 contains little or no sulfur dioxide gas. At this stage the scavenger is regenerated and ready for use in the removal of thiol impurities from a hydrocarbon stream. As in the case of the oxidation stage of the regeneration, it is desirable to avoid a temperature excursion in the reactor, and to this end nitrogen containing but a few volume percent of hydrogen is employed for the initial stages of the reduction, the hydrogen concentration being increased with time. A temperature of the order of 188° C. and a pressure in the range 5.4-6.4 atmospheres is suitable for the reduction stage. Reasonably higher and lower temperatures and pressures may also be employed.

#### EXAMPLES

45 The following examples are submitted for the further demonstration but not the limitation of the invention.

##### EXAMPLE 1

In this example the effective removal of thiol impurity from a cracked gasoline boiling in the 93° C.-177° C. range is demonstrated. This gasoline contained 1.2 ppm of sulfur which was nearly all present as thiol impurity. The scavenger employed was copper chro-

mite disposed upon porous alumina having a surface area of about 180 m<sup>2</sup> per gram. It contained 14 and 3.4 weight percent of copper and chromium, respectively, calculated as the metals. The contacting of the gasoline with the scavenger was at a temperature of about 165° C., a pressure of about 11 atmospheres and a liquid hourly space velocity (LHSV) of about 10. For a period of over 900 hours, the effluent product stream contained no detectable thiol impurity and the non-thiol sulfur-impurity content of this product was less than 0.1 ppm. Thereafter the thiol content of the product stream increased rapidly, indicating that the thiol end point of the scavenger had been reached. At the time of the thiol breakthrough, the scavenger contained 1.2 weight percent sulfur based on the absorbent.

#### EXAMPLE 2

Example 1 was repeated except that the LHSV was increased to 40. As in Example 1, the effluent product stream contained no detectable thiol impurity. The thiol breakthrough was experienced after about 580 hours on stream and the spent scavenger contained 2.25 weight percent sulfur.

#### EXAMPLE 3

Using a scavenger as described in Example 1, a sulfur-containing C<sub>5</sub>-127° C. naphtha was used as the feed. It had a total sulfur content of 340 ppm, of which 58 ppm was in the form of thiol impurity. The contact conditions included a pressure sufficient to maintain the feed in the liquid phase, i.e., of 14.6 atmospheres, an LHSV of 1.0 and a temperature of 260° C. The effluent product stream contained no detectable thiol impurity until breakthrough, which occurred after about 350 hours on stream. At this time the spent scavenger contained about 2.7 weight percent of sulfur.

#### EXAMPLE 4

Example 3 was repeated except that the feed was a C<sub>5</sub>+ -71° C. naphtha having a total sulfur content of 190 ppm, of which 83 ppm was in the form of thiols. The thiol breakthrough occurred after about 270 hours on stream, at which time the spent scavenger contained about 2.7 weight percent sulfur.

#### EXAMPLE 5

Example 4 was repeated except that the contact temperature was 149° C. The thiol breakthrough again occurred after about 270 hours, at which time the spent scavenger contained about 2.4 weight percent of sulfur. After the breakthrough, the rate of increase in the thiol content of the effluent stream was markedly slower than in the case of Example 4.

#### EXAMPLE 6

Example 4 was repeated except that the contact temperature was 93° C. As in the previous Examples 4 and 5, the effluent product stream contained no thiol impurity except that even after 360 hours on stream no thiol breakthrough had occurred. On the other hand, after only 150 hours on stream the sulfur content of the effluent stream increased rapidly and approximated that of the feed. Therefore, rather than absorbing thiol, the scavenger was catalyzing thiol conversion to some other sulfur-containing material, apparently organic disulfides.

#### EXAMPLE 7

Example 4 was repeated except that the feed contained 550 ppm of sulfur of which 110 ppm was in the form of thiol sulfur. The thiol breakthrough occurred after about 190 hours on stream at which time the sulfur content of the spent scavenger was about 2.3 weight percent.

The above examples demonstrate that the conditions of the present process may vary widely: (1) a suitable temperature for the contacting is one which is substantially above 95° C.; (2) the absorption of thiols is rapid, and is effectively accomplished over a wide range of LHSV values; and (3) the presence of a substantial amount of sulfur-containing impurity in the feed other than thiols, while undesirable, does not interfere unduly with thiol absorption by the subject scavengers. The composition of the carrier component may vary widely, provided that it is porous and presents a substantial surface area for the disposition of absorbent scavengers comprising copper. The hydrocarbon feed stream may contain a minor amount of water or water vapor. Preferably the contacting of the hydrocarbon with the scavenger is carried out under substantially anhydrous conditions, that is, in the presence of little or no water. Water in a minor amount, such as is ordinarily present in a conventional hydrocarbon hydroprocessing product stream, does not appear to interfere with the desired thiol absorption.

What is claimed is:

1. A process for absorbing thiol impurity from a hydrocarbon oil boiling in the range from about 10° C. to 300° C. and having a total sulfur-containing-impurity content, calculated as elemental sulfur, below 1000 ppm, including at least 0.4 ppm of thiol impurity, which comprises contacting said oil in the substantial absence of molecular oxygen with a scavenger at a temperature in the range 120° to 400° C., said scavenger comprising an essentially oil insoluble solid composite having a copper component and an inorganic porous carrier component, and having a surface area in the range from about 20 to 1000 square meters per gram, said copper component being copper metal, a copper compound or a mixture thereof, said carrier being a porous inorganic refractory metal oxide or a mixture of such oxides or carbon, and said contacting being continued until the resulting oil product from said contacting has a thiol content below about 0.3 ppm.

2. A process as in claim 1 wherein said copper component is selected from the group consisting of copper metal, copper oxides and copper compounds convertible to copper oxides by ordinary calcining and/or oxidation.

3. A process as in claim 1 wherein said carrier component consists essentially of alumina.

4. A process as in claim 1 wherein said carrier component consists essentially of carbon.

5. A process as in claim 1 wherein said thiol impurity has a carbon atom content in the C<sub>5</sub>+ range.

6. A process as in claim 1 wherein said contacting is at a temperature in the range from about 130° to 200° C. and the thiol content of said oil product is below about 0.2 ppm.

7. A process as in claim 1 wherein said contacting is at a temperature of about 165° C.

8. A process as in claim 1 wherein said contacting is at a pressure sufficient to maintain at least the major portion of the feed in the liquid phase.

9. A process as in claim 1 wherein said scavenger is copper chromite.

10. A process as in claim 1 wherein said scavenger contains an amount of the copper component, calculated as copper metal, in the range from about 1 to 20 weight percent.

11. A process as in claim 1 wherein said composite contains an oxidizing component selected from the group consisting of the oxides of chromium and molybdenum.

12. A process for removing thiol impurity from a gasoline naphtha having a thiol impurity content, calcu-

lated as elemental sulfur, in the range from about 1.2 to 3.0 ppm, which comprises reducing said sulfur content to about 0.1 ppm by contacting said naphtha in the substantial absence of molecular oxygen gas with a scavenger at about 165° C., said scavenger consisting essentially of copper chromite disposed upon alumina having a surface area of about 200 square meters per gram.

10 13. A process as in claim 12 wherein after said contacting is discontinued, said scavenger is regenerated.

\* \* \* \* \*